

E. B. COBB.  
PROCESS OF DESULFURIZING PETROLEUM OILS.  
APPLICATION FILED MAR. 13, 1919.  
**1,357,224.**

Patented Nov. 2, 1920.

2 SHEETS—SHEET 1.



WITNESS:

*Geotekhney*

INVENTOR.

*Ernest B. Cobb*  
BY  
*Safford & Bell*  
his ATTORNEYS

E. B. COBB.  
 PROCESS OF DESULFURIZING PETROLEUM OILS.  
 APPLICATION FILED MAR. 13, 1919.  
**1,357,224.** Patented Nov. 2, 1920.  
 2 SHEETS—SHEET 2.



WITNESS:

*Geo. C. Cheney.*

INVENTOR.

BY *Ernest B. Cobb*  
*Gifford & Bell*  
 ATTORNEY.

# UNITED STATES PATENT OFFICE.

ERNEST B. COBB, OF JERSEY CITY, NEW JERSEY, ASSIGNOR TO STANDARD OIL COMPANY, A CORPORATION OF NEW JERSEY.

## PROCESS OF DESULFURIZING PETROLEUM-OILS.

1,357,224.

Specification of Letters Patent.

Patented Nov. 2, 1920.

Application filed March 13, 1919. Serial No. 282,287.

To all whom it may concern:

Be it known that I, ERNEST B. COBB, a citizen of the United States, residing at Jersey City, in the county of Hudson and State of New Jersey, have invented certain new and useful Improvements in Processes of Desulfurizing Petroleum-Oils, of which the following is a specification.

My invention relates to new and useful improvements in processes for the removal of elementary sulfur from petroleum oils, and my present application is a division, in part, of my prior application, Serial No. 50,177, which was filed in the Patent Office on or about September 11, 1915, Patent No. 1,300,816, which was issued April 15, 1919. By elementary sulfur, I mean that sulfur which exists in the oil in its elementary forms, such as brimstone, flowers of sulfur and all other modifications of elementary sulfur held in physical solution in the oil. The invention is applicable to, and covers the removal of elementary sulfur primarily existing as such in the oil, and also elementary sulfur resulting from acid treatment of the oils, and other processes of refining and chemical treatment. The presence of elementary sulfur in petroleum oils may be ascertained by first testing the oil by any of the well-known tests for hydrogen sulfid or sulfurated hydrogen ( $H_2S$ ) and removing the same, if any be present, by any of the well-known processes for this purpose, after which a piece of bright copper or silver is immersed in the oil freed of sulfureted hydrogen ( $H_2S$ ), and the oil heated; if any elementary sulfur is present it will act to tarnish or blacken the copper or silver. The removal of sulfureted hydrogen from the test oil is a necessary preliminary, because it also darkens copper and silver. But in the treatment of the main body of oil, as hereinafter described, it is unnecessary to remove the sulfureted hydrogen by preliminary treatment.

My present application relates to the removal of elementary sulfur existing in petroleum oils, either primarily, or as the result of treatments or reaction with other compounds or elements, preferably under agitation, by treating the oil with hydroxids of either the alkali metals, particularly sodium, or the alkaline earth metals, particularly calcium, and with hydrogen sulfid. The hydroxids form with the hydro-

gen sulfid monosulfids, and possibly other sulfids. It is well known that higher sulfids of these metals, such as sodium and calcium exist, and the chemical action in using the sulfids resulting from the reaction between the hydroxids and the hydrogen sulfid, as contemplated by my invention, is to cause removal of the elementary sulfur apparently by simple addition, the sulfur combining with the low sulfid of the alkali metal or alkaline earth metal to produce higher sulfids.

My present invention, therefore, contemplates the treatment of the oil with a hydroxid of either an alkali metal or an alkaline earth metal, and with hydrogen sulfid.

In referring to alkaline hydroxids, I include the hydroxids of the alkali metal group, including ammonia, potassium, sodium, and other metals of said group. In practice, I prefer to employ sodium, as it is the most abundant of the metals of this group, and lower in price. Whether the oil is to be treated with hydroxids of the alkali metals and hydrogen sulfid, or whether it is to be treated with hydroxids of the alkaline earth metals and hydrogen sulfid, depends to some extent upon the character of the oil to be treated, the character of the finished products, and the individual preference. By alkaline hydroxids, as used herein, and in the appended claims, I include the hydroxids of the alkali metal group, and the alkaline earth metal group.

The invention is capable of being practised by a variety of apparatus, but, in the accompanying drawings, I have illustrated two types of apparatus which have been successfully used by me.

In the accompanying drawings which illustrate suitable apparatus by which the processes embodying my invention may be carried out, Figure 1 is a view in elevation, partially in section, of an apparatus particularly useful in the practice of my invention when employing hydroxids of the alkali metal group, and hydrogen sulfid, and Fig. 2 is a view similar to Fig. 1, illustrating an apparatus suitable for carrying out my invention when employing hydroxids of the alkaline earth metals, and hydrogen sulfid.

I will first describe the apparatus illustrated in Fig. 1 of the drawings, and then

the method of desulfurizing carried out thereby, after which I will describe the apparatus of Fig. 2, and the method carried out thereby.

5 Referring first to Fig. 1:

1 designates a cylinder or receptacle adapted to receive the oil to be treated, and having a conical bottom 2 and a dome-shaped top or cover 3, provided with explosion doors 31. The conical shaped bottom 2 is provided at its apex with an outlet pipe 4 having a valve 5 at its lowermost portion through which pipe the contents of the cylinder may be flowed when the valve is open, 15 as will be hereinafter described.

6 designates a receptacle or tank of any suitable construction adapted to receive the supply of chemical with which the oil is to be treated, said tank being connected by an 20 outlet pipe 7 with the inlet side of a circulating pump 8, said pipe containing a valve 9 for cutting off and establishing flow through the same to the pump. Connected to the outlet side of the pump is a feed pipe 25 10 extending upward from the pump and provided with a horizontal portion 11 entering the side of the cylinder 1 and provided at its end within the cylinder, with a depending pipe 12 having its lower end closed, 30 but its sides perforated so as to distribute the chemical in fine streams within the cylinder to insure proper admixture of the same with the oil contents of the cylinder. The pipe 7 is connected at a point between 35 the valve 9 and the inlet of the pump to one end of a pipe 13, the opposite end of which is connected to the pipe 4 at a point above the valve 5, heretofore mentioned. The pipe 13 is provided with controlling valves 13<sup>a</sup> 40 and 14 by means of which communication through said pipe 13 to the pump is controlled. Connected at one end to the pipe 4 between the valve 5 and the point of connection of the pipe 13 is an outlet or drain 45 pipe 15 provided with an outlet neck 16 discharging into the tank 6; heretofore described. The pipe 15 is provided with a controlling valve 17 for controlling flow therethrough.

50 18 designates a steam inlet pipe entering through the dome 3 and provided with a depending outlet portion 19 by means of which live steam may be admitted to the interior of the cylinder, an air inlet pipe 20 55 being connected with pipe 18 and provided with a valve 21 for a purpose to be presently described. The pipe 18 may be provided with a valve 22 for controlling the flow of the steam to the same to the interior of the cylinder, said pipe 20 being connected with the pipe 18 between the valve 22 and the outlet end of said pipe 18. Also connected to the steam pipe 18 is a pipe 23 leading to a closed heating coil 24, of any suitable form,

located within the bottom portion of the 65 cylinder, said coil being provided with a control valve 25 for controlling the flow therethrough. The outlet end of the steam coil is shown at 26.

The inlet pipe for feeding the oil to be 70 treated, to the cylinder, is shown at 27, the said pipe entering the cylinder adjacent the upper portion thereof, and extending to a point preferably within the area of the cone-shaped bottom. The treated oil may be 75 withdrawn from the cylinder through an outlet pipe 28, controlled by a valve 29, said pipe being located adjacent to, but above, the lowermost portion of the cone-shaped bottom. The hydrogen sulfid is introduced 80 to the oil from any suitable source through a pipe 30, the end of which extends a short distance, for example, about a foot beneath the surface of the oil to be treated. The pipe 30 is provided with a suitable valve 30'.

I do not desire to be limited in any way to an apparatus such as described, having only described the same in detail so as to insure an adequate understanding of the 90 process embodying my invention.

I will now proceed to describe the process of treating the petroleum oils with hydroxids of the alkali metal group and hydrogen sulfid, this treatment being particularly applicable, but not necessarily confined to 95 paraffin wax, kerosene oil, and white paraffin oil for medicinal use, and I will describe the invention for the sake of illustration for the removal of elementary sulfur from partially finished white medicinal oil.

Previous to treatment this oil may contain .03 per cent. sulfur, of which .02 per cent. is elementary sulfur and .01 per cent. is in the form of inodorous sulfur, not elementary, and in this form unobjectionable 10 in oils for the use stated and contained in sulfur compounds left after treatment with sulfuric acid, said oil being pumped into the vessel or cylinder 1 through the pipe 27. When a sufficient amount of the oil has 11 been charged into the receptacle 1—for instance, in practical operations I have treated 100 barrels of 50 gallons each, when about two-thirds full—steam is admitted into the heating coil 24, and is continued until the 12 temperature of the oil rises to a point where the chemical or chemicals to be added to the oil are active. It will be understood that this is done because chemicals, such as are employed, act slowly at normal temperatures, and rapidly at higher temperatures, and, if the temperature is too low, the operation will become too tedious, and, if on the other hand, the temperature is too high, the oil may become scorched, giving rise to objectionable odor and taste. I prefer to employ a temperature between 160° F. and 190° F., which temperature will usually be

reached within an hour after steam is first admitted to the heating coil, but the time depends largely upon the area of the heating coil.

5 While the preliminary heating of the oil is going on, the chemicals used in the treatment of the sulfur-bearing oil may be mixed in the tank 6, and for this purpose, I preferably employ the following proportions, 10 which I have found give excellent results, but it will be understood that they may be varied as conditions and qualities of the oil may require, or may be deemed expedient, without departing from the spirit of 15 my invention.

To 158 pounds of caustic soda is added 458 pounds of water to form a solution. The caustic soda not only unites with the hydrogen sulfid, in the manner hereinafter described, to form sodium sulfid, but the caustic soda also goes to (1) neutralize any acid bodies left in the oil from previous refining processes, and (2) insures alkalinity to the solution. The solution of the sodium sulfid resulting from the treatment of the oil with sodium hydroxid and hydrogen sulfid appears to be more active when the same is carried out under alkaline conditions.

More water may be added than is indicated, but a longer time will then be necessary to complete the operation. If less water is added, the difficulty of getting a thorough incorporation of oil and the treating solution is increased.

35 When the oil has been raised to the proper temperature, namely, a temperature of 160° F. to 190° F., the solution of caustic soda is injected into the oil within the cylinder. In order to accomplish this, the chemical is 40 drawn through the pipes 7 to the pump 8, and is discharged from the latter through the pipes 10 and 11, and perforated spray nozzle 12, into the oil. It is important, although not essential, to have the chemical 45 in the pipes 10, 11, and spray nozzle 12 under pressure which will be continuous through said pipes up to the perforations in the nozzle, so that the jets of the chemical issuing from the latter will strike the oil 50 with considerable force, and effect a thorough mingling of the oil and the chemical solution.

The chemical solution injected into the oil in the manner described, will gradually 55 find its way by gravity through the body of oil to the bottom of the agitator, and during the initial treatment, I maintain the valves 13<sup>a</sup>, 5 and 17 closed, so that the solution will accumulate in the bottom of the agitator, 60 and the pumping is continued until all, or the desired amount, is drawn from the pipe 6 and injected into the agitator. When the desired amount of chemical solution has been fed to the oil, the valves 13<sup>a</sup> and 14 are

opened, and the valves 5, 9 and 17 closed, 65 and the pump is then operated to circulate the solution through the body of oil being treated, the pipe 13, the pump, the pipes 10, 11, and spray nozzle 12. At the same time the valve 30' in the pipe 30 is opened, and hydrogen sulfid introduced to the oil. During this circulation, the sodium hydroxid and the hydrogen sulfid are brought into intimate contact, and form sodium sulfid, which in turn, reacts upon the elementary sulfur present in the oil to form higher sulfids of the sodium. In carrying out the process, the amount of elementary sulfur present in the oil should first be determined by analysis, and sufficient sodium hydroxid 80 should be added to the oil, so that when the same reacts with the hydrogen sulfid which is injected into the oil, the sodium sulfid so formed, will react with, and eliminate all of the elementary sulfur from the oil. During 85 this circulation, the temperature of the oil being treated is maintained by means of the coil 24, at a temperature of from approximately 160° F. to approximately 190° F. During the treatment described, test samples 90 of the oil are taken from time to time, said samples being washed with water and filtered through filter paper to remove the last traces of moisture, and are then placed in a test glass with a piece of bright copper, 95 and heated to about 175° F. for about one hour. When the test samples cease to show any discoloration or tarnishing of the copper, this stage of the process is considered finished. It may require from one to three 100 hours, because the solution seems to be more active sometimes than at others, for some reason I have been unable to ascertain.

When the test samples cease to discolor the copper, as above described, the chemical 105 solution is allowed to settle in the conical bottom of the vessel, and the settling is continued for a period of from six to ten hours in order to insure all of the solution being separated from the treated oil. When the 110 maximum separation of the solution is assured by adequate settling, the solution may be drawn off from the vessel and returned to the tank 6 through the pipe 4, the pipe 15, and the discharge 16, and said solution reserved for further use in the treatment of 115 oil.

I then treat the oil to remove therefrom any residual alkaline sulfid which may still be suspended in the oil. I prefer to accomplish this by treating the oil with what is known as a "still wash" either by playing water from a hand-hose onto the surface of the oil, drawing the water off continuously at the bottom of the vessel as the 120 water may settle, or the water may be applied by pumping it through a permanent spray pipe S arranged at the top of the 125

cylinder. This treatment may be followed up by an injection of live steam through the pipes 18, 19. This washing process, including the water wash and the steam, may 5 extend over a period of four hours, but may be done in less or greater time, according to circumstances. Instead of injecting live steam from a boiler into the base of the receptacle, I may pump clear, pure water 10 into the bottom of the receptacle and generate steam therefrom, while in direct contact with the oil by means of a heating coil 24<sup>a</sup> similar to the coil 24. This latter method is sometimes preferable because 15 ordinary boiler steam may contain impurities which will be detrimental to the oil being treated. The oil is then allowed to stand for about ten to twelve hours and the water is carefully drawn off and discharged 20 to any suitable point, as, for instance, a sewer, through the pipe 4. It may be that the treated oil still shows a cloud of moisture, but this may be removed by cutting off the steam flowing through the pipes 18, 25 19, and injecting air from the pipe 20 into the pipes 18 and 19 and into the body of oil. This step of the process may continue for a period of from approximately one to approximately three hours, whereupon the 30 oil is usually found bright, and is considered finished.

In Fig. 2 I have shown an apparatus suitable for carrying out the process embodying my invention when a hydroxid of 35 an alkaline earth metal and hydrogen sulfid are to be used in the treatment of the oil.

The apparatus here shown, is the same as that shown in Fig. 1, with the exception 40 that the pump 8, and the connections associated therewith, namely, the tank 6, pipes 7, 13, 10, 11 and 12, for introducing the chemicals to the oil, are dispensed with, since the alkaline earth sulfids which are 45 used in solid form, may be introduced to the oil, for example through the explosion doors 31. Furthermore, the device for introducing water into the oil for washing the same, is unnecessary when the hydroxids of the alkaline earth metals and hydrogen sulfid are used. Furthermore, the process is preferably carried out at a temperature higher than that at which the process using a hydroxid of an alkali metal 50 is carried out, and for the purpose of bringing the metal to the desired temperature, heating coils 24 and 24<sup>a</sup> are provided at their free ends with valves 26' and 24<sup>b</sup>, respectively, which are opened during the 55 heating process just sufficient to permit the condensed water to drain from the device. The pipe 30, which extends a short distance, preferably about a foot beneath the surface of the liquid is provided for introducing hydrogen sulfid to the liquid from 60 65

any suitable source, the pipe being provided with a suitable valve 30'.

Material suitable for carrying out the process with a hydroxid of an alkaline earth metal may be prepared as follows:— 70

800 pounds of freshly burned lime may be placed in an open pan or receptacle, into which is poured 50 gallons of water, the amount of water added being just sufficient to leave the lime in the proper physical condition, neither dusty nor pasty. The oil is first heated to the desired temperature, preferably to a temperature above the condensing point of water, and at a temperature ranging from 212° F. to 300° F. 80 The heating operation is carried out by means of the heating coils 24 and 24<sup>a</sup>, the parts 26' and 24<sup>b</sup> being open sufficiently to permit the condensed water to escape. When the oil has reached the desired temperature, the slaked lime is introduced to the oil in any desired manner, and steam then permitted to pass into the oil through the pipe 19, and thus agitate the oil and bring the hydroxid of the alkaline earth 85 into thorough contact with the hydrogen sulfid, and reacts therewith to form an alkaline earth sulfid. The sulfid in turn reacts with the elementary sulphur present in the oil and forms therewith higher sulfids, and thus eliminates the elementary sulfur from the oil. After the oil has been thoroughly agitated with the calcium hydroxid, the oil is permitted to settle, and the settling will usually require about six hours. The oil 90 is then tested with copper, to determine whether all of the elementary sulfur has been eliminated, and if elementary sulfur remains in the oil, then more hydroxid and hydrogen sulfid must be added, and the 95 process repeated.

What I claim and desire to secure by Letters Patent of the United States is:—

1. The process of removing elementary sulfur from petroleum oil, which consists in 100 treating said oil with an alkaline hydroxid and hydrogen sulfid.

2. The process of removing elementary sulfur from petroleum oil, which consists in 110 treating said oil with an alkaline hydroxid and hydrogen sulfid, and continuing the treatment until the treated oil ceases to have a darkening effect on metallic copper.

3. The process of removing elementary sulfur from petroleum oil, which consists in 120 treating said oil with an alkaline hydroxid and with hydrogen sulfid accompanied by heat at a temperature of from 160° F. to 190° F.

4. The process of removing elementary 125 sulfur from petroleum oil, which consists in treating said oil with an alkaline hydroxid and hydrogen sulfid under alkaline conditions.

5. The process of removing elementary 130

sulfur from petroleum oil, which consists in treating said oil with a solution of an alkaline hydroxid and hydrogen sulfid.

6. The process of removing elementary sulfur from petroleum oil, which consists in treating said oil with a solution of an alkaline hydroxid and hydrogen sulfid, and circulating said solution through the body of petroleum oil.

10 7. The process of removing elementary sulfur from petroleum oil, which consists in treating said oil with a solution of an alkaline hydroxid and hydrogen sulfid, and circulating said solution through the body of petroleum oil until the treated oil ceases to have a darkening effect on metallic copper.

8. The process of removing elementary sulfur from petroleum oil, which consists in treating said oil with a solution of sodium hydroxid in the proportion of about 158 parts by weight of caustic soda and 458 parts by weight of water and with hydrogen sulfid.

25 9. The process of removing elementary sulfur from petroleum oil, which consists in heating said oil for approximately one hour, treating the same with a solution of an alkaline hydroxid and hydrogen sulfid for from approximately one hour to approximately three hours, separating the sulfid resulting from the treatment from the oil, and after-treating the oil to remove residual sulfid suspended in the oil.

30 10. The process of removing elementary sulfur from petroleum oil, which consists in

heating said oil for approximately one hour, treating the same with a solution of an alkaline hydroxid and hydrogen sulfid for from approximately one hour to approximately three hours, while maintaining the same at 40 a temperature of from about 160° F. to 190° F., separating the sulfid so formed from the oil, and after-treating the oil to remove residual sulfid suspended in the oil.

11. The process of removing elementary 45 sulfur from petroleum oil, which consists in heating said oil to a temperature of from about 160° F. to 190° F., treating the same with a solution of an alkaline hydroxid and hydrogen sulfid, separating the sulfid 50 formed by the treatment from the oil, and after-treating the oil to remove residual sulfid suspended in the oil.

12. The process of removing elementary sulfur from petroleum oil, which consists in 55 treating said oil with an alkaline hydroxid and hydrogen sulfid accompanied by agitation.

13. The process of removing elementary sulfur from petroleum oil, which consists in 60 treating said oil with an alkaline hydroxid and hydrogen sulfid accompanied by agitation and heat.

In testimony whereof I have hereunto signed my name in the presence of two sub- 65 scribing witnesses.

ERNEST B. COBB.

Witnesses:

ADELE S. EBERHARDT,  
DANN L. Wood.